

Sept. 29, 1925.

1,555,520

J. A. SCHAEFFER ET AL

METHOD AND APPARATUS FOR MANUFACTURING BASIC LEAD SULPHATE PIGMENT

Filed May 22. 1924



Inventors.

John A. Schaeffer  
John H. Calbeck  
Bernard S. White

by Francis J. Chambers  
their Attorney

Patented Sept. 29, 1925.

1,555,520

## UNITED STATES PATENT OFFICE.

JOHN A. SCHAEFFER, OF ST. LOUIS, AND JOHN H. CALBECK AND BERNARD S. WHITE, OF JOPLIN, MISSOURI, ASSIGNEES TO THE EAGLE-PICHER LEAD COMPANY, OF CINCINNATI, OHIO, A CORPORATION OF OHIO.

### METHOD AND APPARATUS FOR MANUFACTURING BASIC-LEAD-SULPHATE PIGMENT.

Application filed May 22, 1924. Serial No. 715,016.

*To all whom it may concern:*

Be it known that we, JOHN A. SCHAEFFER, citizen of the United States of America, and resident of St. Louis, county of St. Louis, State of Missouri, and JOHN H. CALBECK and BERNARD S. WHITE, citizens of the United States of America, and residents of Joplin, county of Jasper, State of Missouri, have invented certain new and useful Improvements in Methods and Apparatus for Manufacturing Basic-Lead-Sulphate Pigment, of which the following is a true and exact description, reference being had to the accompanying drawings, which form a part thereof.

Our invention relates to the manufacture of a fumed basic lead sulphate pigment and has for its object the production of such a pigment of high and uniform quality. Fumed basic lead sulphate pigment, as heretofore commercially produced, has generally been made in an apparatus comprising one or more low cupola furnaces, a hot flue or combustion chamber into which these furnaces deliver the fume and gas, a tower into which the combustion chamber opens and which in turn delivers the gases and fumes to a cooling system through which they are drawn by a fan, and which fan finally forces the gas and fume into a screen system of the screen bag type. This method and apparatus is fully described in the patent to Bartlett 515,040 of February 20, 1894. The pigment produced in this way and by this apparatus is of good average quality and color but at times is so off color that it has been found advisable to refurnace the fumes in order to keep up the standard qualities of the pigment, and this, of course, adds materially to the expense of the process.

Recently we have succeeded in manufacturing a basic lead sulphate pigment of a whiteness, brightness and covering power greatly better than the product of the process and apparatus we have described, by a method in which we project atomized lead into a heated furnace having an atmosphere containing oxygen and sulphur dioxide gas in such proportionate quantity to the lead as to form with it a basic lead sulphate of the desired composition. This method forms the subject matter of our pending applica-

tion for Letters Patent, Serial No. 626,278, filed March 20, 1923, and the new pigment produced by this process, forms the subject matter of our pending application, Serial No. 655,242, filed August 2, 1923, said new pigment being characterized, in addition to its distinctive characteristics, by having a high percentage of combined lead oxide and substantially no uncombined lead oxide.

Our new process consists in mixing fume and furnace gases from the low cupola system with the fume and furnace gases issuing from the furnace in which the atomized lead is treated, as described, thoroughly mixing the products of both furnaces together by passing them through a fan and forcing the mixed product into a screen system for the separation of the fumed basic lead sulphate. This process results in a homogeneous, high quality, basic lead sulphate, the color of which can be nicely regulated and brought to standard by regulating the percentage of admixture of the two furnace products, and it will readily be understood that the percentage of the fume coming from the furnace in which the atomized lead is treated, can be regulated with the atomized oxide so as to correct any temporary color deficiencies in the product of the low cupola furnace. Our process will be best understood as described in connection with the drawing which diagrammatically illustrates the apparatus which we have invented for carrying it into effect, and which apparatus also forms the feature of our invention.

A, A, indicate the low cupola furnaces. B, the combustion chamber into which they open. C, the combining tower. D, the cooling system; E, the fan which draws the gases from the cooling system and delivers them into a main F, from which, in turn, they pass through the branches F' into the screen system, indicated at G. H indicates the furnace for the treatment of atomized lead. I, a lead kettle from which melted lead is sprayed into the furnace H by an atomizer indicated at J. K indicates a conduit through which sulphur dioxide gas is introduced into the same end of the furnace into which the lead is projected. L is a combustion chamber connected with the furnace H and connecting through a main M,

a cyclone fan indicated at N, and a conduit O, with the screen system indicated at D. P is a damper in the conduit O.

In operation, lead ore and lead products containing sulphur in sufficient quantity are treated in the low cupola furnaces A, with the result that each of their lead contents is driven off as a basic lead sulphate fume, which, together with the furnace gases, pass into the combustion chamber B and into the tower C, from which these gases and fumes pass to the cooling system D, and through the fan E, into the bag room. At the same time, atomized lead is projected into the furnace H where it is exposed to the action of oxygen and sulphur dioxide gas in quantity to combine with the lead and form a basic lead sulphate of the desired composition. The fume and gases from the furnace H pass through the combustion chamber L, through the fan N and conduit O into the cooling system, where they mix with the products of the low cupola furnaces, the mixture being insured and made thorough by the action of the fan E, through which the mixed products are passed so that the material passing from the fan into the screen system is of uniform combustion.

It will readily be understood that by regulating the amount of atomized lead fed to the furnace H and also by the manipulation of the damper P, any desired percentage of the distinctive new pigment can be fed to the cooling system and into admixture with the products of the low cupola furnace and in this way the production of a basic lead sulphate of very high and uniform quality can be insured even when the low cupola system is not working to give its best results.

Having now described our invention, what

we claim as new and desire to secure by Letters Patent, is:

1. The method of manufacturing a basic lead sulphate pigment of high and uniform quality which consists in treating lead ores and products containing sulphur in low cupola furnaces for the production of a basic lead sulphate fume, drawing the gas and fume from said furnaces through a system of hot flues and cooling means by the action of a fan, simultaneously spraying atomized lead into a heated furnace chamber having an atmosphere containing oxygen and sulphur dioxide gas in quantity to combine with the atomized lead and produce a basic lead sulphate fume thoroughly mixing the fumes and gases from the two furnaces and separating the basic lead sulphate fume from the mixed furnace gases by screening. 50 55

2. Apparatus for the manufacture of basic lead sulphate pigment comprising in combination one or more low cupola furnaces for treating lead ores and products containing sulphur, for the production of basic lead sulphate fumes, a cooling system, a screen system, a fan for drawing the fume and gas from the furnaces through the cooling system and forcing them into the screen system, a separate furnace adapted to treat atomized lead in an atmosphere of oxygen and sulphur dioxide gas for the production of basic lead sulphate fume, and a conduit connecting said separate furnace with the flue system of the low cupola furnace at a point where the gases and fumes will mix before passing through the fan and into the screen system. 60 65 70 75

JOHN A. SCHAEFFER.

JOHN H. CALBECK.

BERNARD S. WHITE.